

March 28, 1933.

**H. B. ARDEN**

**1,902,937**

## METHOD FOR AUTOMATIC ELECTROMAGNETIC WET SEPARATION

Original Filed Oct. 11, 1928 4 Sheets-Sheet 1



Fig. 2.

Fig. 1.

Fig. 3. INVENTOR:  
Harry B. Arden  
BY  
O. W. Edwards  
his ATTORNEY.

March 28, 1933.

H. B. ARDEN

1,902,937

METHOD FOR AUTOMATIC ELECTROMAGNETIC WET SEPARATION

Original Filed Oct. 11, 1928 4 Sheets-Sheet 2



Fig. 4.

Inventor:  
Harry B. Arden

By his Attorney

O. Cleary Edwards

March 28, 1933.

H. B. ARDEN

**1,902,937**

## METHOD FOR AUTOMATIC ELECTROMAGNETIC WET SEPARATION

Original Filed Oct. 11, 1928 4 Sheets-Sheet 3



Fig. 6.

Fig. 5.

Inventor:  
*Harry B. Arden*

By his Attorney

His Attorney  
O. E. Kelly

March 28, 1933.

H. B. ARDEN

1,902,937

METHOD FOR AUTOMATIC ELECTROMAGNETIC WET SEPARATION

Original Filed Oct. 11, 1928 4 Sheets-Sheet 4



Inventor:  
Harry B. Arden

By his attorney  
O. G. Edwards

## UNITED STATES PATENT OFFICE

HARRY B. ARDEN, OF NEW YORK, N. Y.

## METHOD FOR AUTOMATIC ELECTROMAGNETIC WET SEPARATION

Application filed October 11, 1928, Serial No. 311,869. Renewed February 24, 1932.

The object of my invention is to provide a method which may be used to separate the magnetic from the non-magnetic matter carried with a downwardly flowing stream 5 of water. The magnetic substance may be in finely crushed ore, the magnetite of black sand deposits, or any other finely divided magnetic substance which can be carried within a stream of water. This and other 10 objects are accomplished by my invention, some embodiments of which are hereinafter more particularly set forth.

For a more detailed description of my invention, reference is to be had to the accompanying drawings, forming a part hereof, in 15 which

Figure 1 is a front elevation of one embodiment of my invention.

Figure 2 is a similar view with the feed 20 hopper and stream guides removed.

Figure 3 is a side elevation of the structure shown in Figure 1.

Figure 4 is an enlarged sectional view of 25 a portion of the apparatus shown in Figure 3.

Figure 5 is a front elevation of a multiple apparatus to be used for a double separation.

Figure 6 shows the front plate and ore 30 ducts of a modification of the apparatus shown in Figure 1, which is to be used to segregate the strongly from the weakly magnetic substances.

Figure 7 shows a further modification 35 wherein but one feed hopper is used with one long stream guide.

Figure 8 shows a front view of the hopper and stream guide shown in Figure 7.

Figure 9 is a sectional view, taken on the line 9—9 of Figure 8.

40 Figures 10 to 14 inclusive show details of my improved hopper and stream guide, Figure 11 being a sectional view, taken on the line 11—11 of Figure 10; Figure 12 is a top plan view of a hopper and Figures 13 and 45 14 are bottom views of stream guides, Figure 14 differing from Figure 13 only in having side walls converging slightly, as shown.

Figure 15 is a diagrammatic view of the 50 electrical connections and circuits.

Throughout the various views of the draw-

ings, similar reference characters designate similar parts.

My improved method employs a separating apparatus 11 which is provided with a mixture 17 of water and magnetic ore bearing material, fluid enough to flow freely, which is supplied through the pipes 12 and is controlled in quantity by the valves 13, passing therefrom through outlets 14 into the top hoppers 15 and through narrow passages 19 at the bottom of the hoppers, which passages join the stream guides 16, which guide the stream down their inner surfaces and into the next lower hoppers 15.

The fluid mixture of ore and water from the outlets 14 into the top hoppers 15 should be in sufficient quantity to fill the hoppers so that an overflow will occur at the lips 15a into the overflow tubes 18 attached to the front of each hopper and stream guide, the surplus water going into the next lower hopper to compensate for magnetic substances withdrawn from the stream. This overflow should take place successively from upper to lower hoppers, thus maintaining an even pressure 70 through passages 19, thus assuring a smooth, unbroken downward gliding stream of ore and water within the stream guides 16.

The passages 19 terminate and join with 80 the stream guides 16 which are in the form of shallow troughs having front walls 20 and sides 21, the open backs being toward the magnetic source. These hoppers and stream guides are mounted so that the walls 85 20 are inclined slightly from the vertical, as shown in Figures 3 and 4, the object being to cause the falling stream of ore and water to impinge and flow in a smooth stream within the confines of the stream guides 16.

The walls of the hoppers 15 have hooks 90 15b, or other means provided for attaching them to the ore troughs 22, which are fixed to the front of shield plates 23 which are attached in vertical position to the frames 24 of the apparatus. These ore ducts each have a sloping floor sufficiently inclined to be self clearing when a stream passes over it. Back of the plate 23 are a series of electromagnets designated generically by the character 95 25 and specifically according to the sys-

tems in which they are connected, there being, in the embodiment shown, four of these systems numbered 1 to 4 inclusive, as shown in Figure 15. These magnets are also supported by the frame 24 in any suitable manner, but preferably with their pole pieces against the back of the plate 23, as shown, and they are rigidly mounted and separated from all water by this plate.

10 The support 24, the plate 23, the stream guide 16, the hoppers 15 and the overflow tubes 18, as well as the pipes 12, valves 13 and outlets 14 and all other parts, should be made of non-magnetic material, the only magnetic 15 material that is employed in the apparatus being that of the cores 26 of the magnets 25.

Wash water 27 is supplied through suitable perforated pipes 28 from vertical pipes 29 governed by a valve 30 and one of these

20 perforated pipes 28 is preferably located, as indicated in Figure 4, just above the level of the adjacent magnet 25, so that when the magnet is not energized the abundant flow of water will wash the ore, which is free, or 25 substantially free of silica or other impurities, into the ore duct 22, from whence it is drained through drain pipes 31 into a suitable receptacle 32, where it is received and held ready for further treatment.

30 The magnets 25 are divided into four systems in the embodiment shown, and each system is numbered 1 to 4 inclusive, as above stated, and supplied by electricity from any suitable source, as from a direct current generator 33 and this generator has one pole 34 connected to a wire 35 that runs to the lead in wires 36 of the respective magnets and the other pole 37 of this generator 33 is connected by a wire 38 to brushes 39 which bear

40 on a commutator 40 which has its bars arranged in four series so that every fourth bar is connected to the first system, the next series has every fourth bar connected in the second system, the third series has every 45 fourth bar connected and in a similar manner, the fourth series has every fourth bar connected, and so, in the embodiment shown, the commutator has segments in multiples of four all connected as indicated. The first 50 system is connected to the proper part of the commutator by a wire 41 which runs to a lead in wire of the magnet 1. In a similar manner, the second series has a wire 42 which runs to the lead in wire of the magnet 2 and

55 similarly the third system has a lead in wire 43 and the fourth system a lead in wire 44. The commutator is run in such a way that the magnets are properly energized beginning with 1, 2 and 3, then 2, 3 and 4, then 3, 60 4 and 1, then 4, 1 and 2, so that three are always energized and one is deenergized. The time of energizing each magnet will vary according to the flow and nature of the ore being treated and under the usual conditions 65 of service the time each magnet will be ener-

gized will be substantially three-quarters of a second and it will be deenergized for one-quarter of a second. As long as each magnet is energized it will hold the ore adjacent thereto on the plate 23 and close to its pole pieces 26 and the instant it is deenergized the abundant stream of water 27 will cause it to fall into the ore duct 22, as above stated.

The advantage of having the magnets function in the order above described, is that at all times the material must pass through the magnetic field of an energized magnet and nothing will pass free thereof. If the magnets were energized in the opposite way, it might be that at times ore between 75 systems 1 and 2 would pass free of all magnetism during the instant that the first system is deenergized and thereby permit loss of values.

The lowest overflow tube 18, as well as the lowest stream guide 16, drain into the outlet pipe 45 which carries away the tailings from the apparatus and also the excess water.

In view of the foregoing, the operation of this embodiment of my invention will be readily understood. Assuming that a flow of water is maintained through the pipes 29 and a flow of water and sand bearing ore through the pipes 12 and a suitable electric current passes through the magnets, as above set forth, the action is as follows. The hoppers 15 fill rapidly and immediately the mouths of the outlets 14 are submerged and an overflow into and through the overflow tubes 18 takes place.

As the magnets 25 are successively energized, the ferrous or other magnetic material accumulates on the front of the plate 23 while non-magnetic material is carried into the next lower hopper 15 until the end of the apparatus is reached. The magnetic ore is released the instant the magnet is deenergized and is washed down by the stream 27 into the ore duct 22 from whence it is passed to the drain 31, as above set forth. If some of the magnetic material gets by the first magnet 25, it will be caught by one of the lower magnets in the manner just described, so that after the material has passed the last magnet its separation is practically complete under normal conditions. To further concentrate the separated material, the apparatus described below is employed.

In Figure 5 is shown a modification where-in there are two sets of hoppers 15 and stream guides 16 as well as overflow tubes 18 mounted side by side, all functioning precisely as above described, the waste water and gangue escaping by drain pipes 45, as above set forth. The ore which is caught in the upper ore ducts 22 is passed into a suitable tank 46 provided with agitating jets through nozzles 47 and the excess water is drained from the tank 46 by means of a suitable drain 48 which runs to a pipe 45. From the bot-

tom of the tank 48, pipes 12 run precisely as above described, and the ore is further concentrated by this lower apparatus, precisely as shown in Figure 1.

5 In Figure 6 the ore and water pipes are omitted as well as the troughs 16 and attached parts and only the plate 23 is shown together with the ore ducts 22 which are divided into two series of three each, as 10 appears on the drawings. The upper series is provided with magnets which function exactly as above described, so as to draw off the strongly magnetic material from the stream precisely in the manner above indicated, and this is drained through the pipe 31 into a suitable receptacle 32. The three lower magnets associated with the three lower ore ducts 22 have a much stronger magnetic flux, so as to recover the weaker magnetic material which otherwise would escape, and this drains into a receptacle 49. This embodiment of my invention is useful where it is desired to segregate weakly magnetic material carrying values other than that of 15 iron.

In the embodiment of my invention shown in Figures 7 to 9 inclusive one long stream guide 50 drains the hopper 15 and instead of one plate 23 a series of short plates 51 are 20 employed, each one overlapping the lower, as indicated, and these plates and the stream guide 50 converge towards the bottom of each plate by reason of the slope of the stream guide 50, so that the stream will 25 follow an inclined surface and have a smooth, swift descent through the successive magnetic fields of the magnets. At the bottom the water and sand drain out through a pipe 45 and the ore passes with some water 30 through another pipe 52.

The structure of Figure 14 shows converging side walls which more effectively confine the stream than the straight walls of Figure 13. The advantage is slight but substantial 45 as all tendency of the stream to climb the side walls is thereby eliminated.

While I have shown and described some embodiments of my invention, it is obvious that it is not restricted thereto, but that it 50 is broad enough to cover all methods that come within the scope of the annexed claims.

Having thus described my invention, what I claim is:

1. The method of automatic, electro-magnetic wet separation which consists in passing 55 downwardly a substantially vertical, smooth-flowing stream of magnetic ore and water through an intermittent magnetic field which separates the magnetic from the non-magnetic material carried by the stream.

2. The method of automatic, electro-magnetic wet separation which consists in passing 60 downwardly a substantially vertical, smooth-flowing and controlled stream of magnetic ore and water through intermittent magnetic

fields which separates the magnetic from the non-magnetic material carried by the stream.

3. The method of automatic, electro-magnetic wet separation which consists in passing 65 downwardly a substantially vertical, smooth-flowing stream of magnetic ore and water through an intermittent magnetic field which separates the magnetic from the non-magnetic material carried by the stream and holds the magnetic material momentarily and then washing down such held material immediately upon the release of the magnetism.

4. The method of automatic, electro-magnetic wet separation which consists in passing 70 downwardly a substantially vertical, smooth-flowing stream of magnetic ore and water through successive, intermittent magnetic fields, which operate successively from the bottom up and which separates the magnetic from the non-magnetic material carried by 75 the stream.

5. The method of automatic, electro-magnetic wet separation which consists in passing 80 downwardly a substantially vertical, smooth-flowing stream of magnetic ore and water, through two series of intermittent magnetic fields, of different intensities, the first being the weaker, whereby stronger and weaker 85 magnetic ores may be separated.

6. The method of automatic, electro-magnetic wet separation which consists in passing 90 downwardly a substantially vertical, smooth-flowing stream of magnetic ore and water through intermittent magnetic fields which 95 partially separate the magnetic from the non-magnetic material carried by the stream, and thereafter passing, in the same way, this magnetic constituent through a second series of 100 intermittent magnetic fields.

In testimony whereof, I have hereunto set 105 my hand this 9th day of October, 1928.

HARRY B. ARDEN.

110

115

120

125

130